

July 14, 1925

1,546,346

S. G. MANDALIAN

ENAMELED ARMOR MESH FABRIC AND METHOD OF FINISHING SAME

Filed April 5, 1924

*Fig. 1.*



*Fig. 2.*



*Fig. 3.*



Inventor  
Sahatel G. Mandalian

By  
Horatus E. Bellows  
Attorney

## UNITED STATES PATENT OFFICE.

SAHATIEL G. MANDALIAN, OF NORTH ATTLEBORO, MASSACHUSETTS.

ENAMELED ARMOR-MESH FABRIC AND METHOD OF FINISHING SAME.

Application filed April 5, 1924. Serial No. 704,363.

*To all whom it may concern:*

Be it known that I, SAHATIEL G. MANDALIAN, a citizen of the United States, residing at North Attleboro, in the county of 5 Bristol and State of Massachusetts, have invented certain new and useful Improvements in Enamored Armor-Mesh Fabrics and Methods of Finishing Same, of which the following is a specification.

10 My invention relates to metallic mesh fabric adapted to use in the construction of mesh bags, purses, and other ornamental articles; and particularly to that type of mesh commonly known as "armor mesh" or 15 "fish scale mesh." This type of mesh comprises parallel series of cruciform links or plates each having four corner prongs converging in the rear of the plate and engaging thereby four metal ring links. The 20 front of the metal fabric thus composed has a coating of colored enamel.

The metals which are suitable for this construction are, like brass, German silver, silver plate, and the like, of a bright or shiny 25 character; the different links are jointed and to a limited extent movable with relation to each other; and the top surfaces of ring links lie in a slightly lower plane than those of the plate links. Therefore to attempt 30 a blanket deposit of enamel upon the surface of a mesh strip has not heretofore been commercially feasible because it failed to effectually cover and permanently conceal the joints and occasional ring links, but im- 35 parted to the complete article a tinny, raw, and unfinished, rather than a salable uniform, and soft appearance.

The essential objects of my invention are 40 to remedy the above defects, and attain the recited advantages, as well as, to enable the successful use of more delicate shades of enamel than has been heretofore possible.

To the above ends essentially my invention consists in such parts and combinations, 45 and in such steps and combinations of steps as fall within the scope of the appended claims.

In the accompanying drawings which 50 form a part of this specification

Figure 1 is a front elevation of an armor mesh fabric, greatly enlarged, embodying and made according to my invention,

Figure 2, a section of a cruciform link on line 2—2 of Figure 1, and

Figure 3, a section of a ring link on line 3—3 of Figure 1.

Like reference characters indicate like parts throughout the views.

In carrying out my invention an armored mesh fabric is constructed in the usual manner from German silver, brass, silver plated or nickel plated stock, or other thin bendable metal. This consists of parallel circular or ring links, represented generally by 4, each four of which links are loosely engaged to a flat cruciform link or plate, represented in a general way by 5, by four corner prongs 6 converging in the rear of the plate.

It is sought to apply enamel to this fabric, but in order to attain the results hereinabove referred to I have ascertained that it is necessary to impart a dark finish to the fabric prior to the application of the enamel. This preliminary step of darkening the metal may be effected in various ways, such for instance as dipping the fabric in sodium sulfide solution.

After the darkening step, the enamel of any desired ornamental color is applied to the face of the mesh fabric in an convenient manner. That is to say the enamel in liquid state may be applied to the front face of the fabric and then baked thereon.

In Figure 2 the body of a link 5 is indicated by 7, and the enamel coating thereon by 8. In Figure 3 the body of the link is indicated by 9, and the enamel by 10.

To physically apply the enamel to the fine and flexible fabric is very difficult, and necessarily certain parts of the fabric, such as portions of the ring links 4, do not receive their intended share of enamel. This defect, however, is not apparent because of the darkened condition of the metal stock, and it is thus possible to produce a commercial article, and with speed as well as at small expense.

I claim:—

1. In a metallic mesh fabric for ornamental articles, cruciform links, ring links engaging the corners of the cruciform links, and an enamel coating upon the exposed surfaces of the cruciform links and the ring links.

2. In a metallic mesh fabric for ornamental articles, cruciform links provided with darkened exposed surfaces, ring links

engaging the corners of the cruciform links and provided with darkened exposed surfaces, and an enamel coating upon the exposed surfaces of the cruciform links and 5 the ring links.

3. A method of finishing metallic armor mesh fabric for ornamental articles of inter-engaging constituent metallic links, by darkening the surfaces of the links, and 10 depositing a coating of enamel upon the darkened links.

4. As an improved article of manufacture a metallic mesh fabric having interstices through which portions of the rings of the mesh are visible, the said portions being 15 darkened so that the portions of the rings in such interstices are made less conspicuous, the exposed portions of the mesh being enameled.

In testimony whereof I have affixed my 20 signature.

SAHATIEL G. MANDALIAN.